

Patented Dec. 9, 1924.

1,518,760

# UNITED STATES PATENT OFFICE.

JOSEPH M. SCHWARZ, OF NEW YORK, N. Y.

## ALUMINUM NICKEL ALLOY.

No Drawing.

Application filed August 10, 1922. Serial No. 581,026.

To all whom it may concern:

Be it known that I, JOSEPH M. SCHWARZ, a citizen of the United States, and resident of New York, in the county of New York and State of New York, have invented certain new and useful Improvements in Aluminum Nickel Alloys, of which the following is a specification.

This invention relates to aluminum alloys and has for its main object to provide an alloy of the mentioned type which will have greatly improved physical properties against the alloys of the mentioned character used at the present time. I especially aim to provide an aluminum alloy which will have all the desirable characteristics of such alloys as used at present, mainly in building automobiles, aeroplanes, etc., as for instance, low specific gravity, resistance to acids, and other corrosives, but at the same time, having a greatly increased tensile strength and ductility.

Many aluminum alloys have been invented and used for the above mentioned purposes and they may be divided into three classes: aluminum copper alloys,—aluminum zinc alloys,—and aluminum magnesium alloys. These alloys have the advantage of being comparatively light as against other alloys of metals of similar strength, but nevertheless, their tensile strength, and in many cases, their resisting power, and their adaptability to manufacturing processes, do not come up to the requirements which an alloy in automobile and aeroplane manufacture, or in similar uses would have to meet.

I discovered that by adding a certain amount of nickel to the aluminum copper alloys, a new composition will result which is greatly superior in all the desirable qualities mentioned above and relating to alloys to be used in automobile and aeroplane manufacture as well as for any other machine parts where such qualities are needed. I also discovered that by adding a certain amount of nickel to such alloys, I can materially increase the amount of copper in my alloy without running the danger of obtaining an unworkable or brittle alloy as has been the case with aluminum copper alloys heretofore when the copper content has been increased over 7 or 8 per cent.

My alloy consists of aluminum, a relatively small proportion of copper and of nickel in still smaller amounts. The average amount of aluminum in my alloy is between 85 per cent and 96 per cent; the balance to be made up with copper and nickel in a proportion of 2 for copper and 1 for nickel. By varying these proportions, we may obtain a series of alloys adaptable to different purposes.

I have also discovered a certain method of alloying, as the best adapted to produce my new metal. This process is as follows:

I first melt the copper down and introduce the nickel into it as a hardener. The alloy of these two metals is then poured either into shot-form or into strips of a thickness of about  $\frac{1}{8}$  of an inch. The aluminum is afterwards melted at a temperature of about  $1400^{\circ}$  Fahrenheit, in the usual way, the above mentioned hardening alloy introduced into the aluminum bath and stirred constantly until complete amalgamation takes place. While producing my alloy, I may use an effecient di-oxidizer.

What I claim as new and want to protect by Letters Patent is:

1. The within described alloy, composed of aluminum in a relatively large amount, and relatively small amounts of copper and nickel, the percentage of the aluminum being ninety or more, and the percentages of the copper and nickel being in the proportion of two to one.

2. The within described alloy, consisting of aluminum, 90 to 97 per cent, copper seven and one half to two per cent, and nickel, two and one half to one per cent.

3. The process of producing the within described alloy, consisting in melting down copper, 10 to  $2\frac{1}{2}$  per cent, introducing nickel 5 to  $1\frac{1}{2}$  per cent in the molten copper, and pouring this hardening mixture into shot form or into strips; melting aluminum 85 to 96 per cent, adding the hardener described hereinbefore, constantly stirring until complete amalgamation and using a di-oxidizer.

Signed at New York in the county of New York and State of New York this day of August A. D. 1922.

JOSEPH M. SCHWARZ.